

March 17, 1936.

C. H. DAVIS  
COPPER AND COPPER BASE ALLOYS

2,034,561

Filed Oct. 13, 1934



Fig. 1



Fig. 2



Fig. 12



Fig. 13



Fig. 3



Fig. 4



Fig. 14



Fig. 15



Fig. 5



Fig. 6



Fig. 7



Fig. 8



Fig. 18



Fig. 19



Fig. 9



Fig. 10



Fig. 20



Fig. 11

INVENTOR  
Charles H. Davis  
BY  
Woolster & Davis  
ATTORNEYS.

## UNITED STATES PATENT OFFICE

2,034,561

## COPPER AND COPPER BASE ALLOYS

Charles H. Davis, Cheshire, Conn., assignor to  
The American Brass Company, Waterbury,  
Conn., a corporation of Connecticut

Application October 13, 1934, Serial No. 748,193

2 Claims. (Cl. 138—47)

This invention relates to articles made of copper and copper base alloys improved with respect to resistance to corrosion or intercrystalline partitioning in the metal, particularly in steam, by the addition of a certain amount of cadmium.

It has been found in certain types of steam service, especially at temperatures above 212° F. (100° C.) and pressures above atmospheric, that the steam and (or) gases commonly associated with steam in ordinary manufacturing or commerce cause certain copper base alloys to disintegrate or crack.

Notable failures of copper and copper base alloys have occurred while in use, as portions of expansion joints in the steam lines in large cities, such as New York and Boston. The early or unexpected failure of copper or copper base alloys in these locations is a serious menace to commerce and health. An intensive study of the causes of such failures in copper base alloys was initiated with the result that by a novel method of testing in steam, certain alloys have been discovered to be particularly resistant to the action of steam at elevated temperatures.

The disintegrating action of the steam or gases in the steam mentioned in the previous paragraphs is especially pronounced at the boundaries of the grains of the alloys, separating said grains or crystals by destroying the cohesion and bond that normally holds the alloy crystals together in a strong, unified mass. Certain copper base alloys, when under stress, or when alternately stressed and unstressed, have been shown more susceptible to this disintegrating action of steam and (or) gases in steam than other copper base alloys. Commercially pure copper itself is susceptible to this action just described and fails quickly under the higher unit stresses.

The effect of steam at elevated temperatures upon copper and certain copper base alloys is known to the engineers in charge of aforesaid steam lines and to certain of the engineering and metallurgical professions, but it has been further demonstrated in a novel method of laboratory test.

Wires of copper and many copper base alloys have been subjected while under stress, or while alternately stressed and unstressed, to the action of steam. It was found by said tests that representative wrought copper base alloys from the following alloy systems, while under stress, are susceptible to a greater or less degree to the disintegrating action of steam, and this indicates the remaining alloys of these systems are also so

susceptible to this disintegrating action. These systems include, in addition to the commercially pure copper:

|                                                                               |    |
|-------------------------------------------------------------------------------|----|
| Commercial copper-silicon alloys up to at least 4% silicon                    | 5  |
| Commercial copper-aluminum alloys                                             |    |
| Commercial copper-silicon-manganese alloys                                    |    |
| Commercial copper-zinc alloys                                                 |    |
| Commercial copper-zinc-nickel alloys                                          | 10 |
| Commercial copper-tin alloys                                                  |    |
| Commercial copper-tin-nickel alloys                                           |    |
| Commercial copper-aluminum-tin alloys                                         |    |
| Commercial copper-zinc-tin alloys                                             |    |
| Commercial copper-nickel alloys                                               |    |
| Commercial copper-nickel-silicon alloys                                       | 15 |
| Commercial copper-zinc-silicon alloys                                         |    |
| Commercial copper-nickel-aluminum-zinc alloys and similar copper base alloys. |    |

A large number of copper base alloys without cadmium and others containing cadmium have been tested, and although the improvement is greater in certain alloys than in others the tests indicate that practically all copper base alloys are improved at least to some extent by the presence of cadmium in the alloy with respect to resistance to corrosion in steam.

The tests were made in a cylindrical steam chamber with normal pressure 130 pounds per sq. in. gauge pressure, equivalent to a temperature of about 180° C. The steam was analyzed and the impurities determined. The copper base alloy specimens were in the form of .036" diameter wire and these passed through glands sealed with asbestos packing in each head of the chamber so that a load of any size might be applied to stress the wires. The loads varied from no load up to 80% of the ultimate strength of the specimens. Tests made under intermediate loads, such as 5%, 10%, 20%, 30%, 40%, etc. of the ultimate strength of the specimens revealed that the length of life of the specimens under test in steam varied proportionally with the amount of load or stress applied during the test. Hence, tests were conducted at stresses both under and over the yield point, elastic limit and (or) proportional limit of many specimens. The usual procedure was to keep the steam turned on at all times but to remove the load for a certain period of each day.

It was found by this novel method of test that certain copper base alloys quickly failed by intergranular separation, beginning at the surfaces of the specimens and extending inward until the

remaining cross-section of sound metal fractured because of the increased unit stress.

Another type of failure was discovered where the grains parted in the interior of the specimens with no apparent connection with the surfaces. Certain specimens failed by one or the other of these types of intergranular separation, while others failed by a combination of the two types of parting.

10 In order to present concrete evidence of the behavior of several selected copper base alloys in the testing apparatus described in the above paragraphs, examples of these alloys are now listed. The specimens were in the steam chamber in about 130 lbs. per sq. in. steam pressure (180° C.) and each specimen was stressed individually to 80% of its ultimate tensile strength.

15 The above actual steam tests and many other similar tests have demonstrated the superiority

20 *Results of tests in steam of various copper bar alloys each stressed to 80% of its ultimate strength*

| No. | Alloy  |     |      |      |      |       |       | Failed at hours under stress |
|-----|--------|-----|------|------|------|-------|-------|------------------------------|
|     | Cu     | Sn  | Cd   | Si   | Mn   | Ni    | Al    |                              |
| 1   | 98.79  |     | 1.20 | .01  |      |       |       | 3266                         |
| 2   | 98.58  | .60 | .80  | .02  |      |       |       | 3002                         |
| 3   | 97.00  |     |      | 3.00 |      |       |       | 1                            |
| 4   | 96.00  |     | 1.00 | 3.00 |      |       |       | 76½                          |
| 5   | 94.00  |     |      |      | 5.00 | 1.00  |       | 160                          |
| 6   | 93.00  |     | 1.00 |      | 5.00 | 1.00  |       | 1699                         |
| 7   | 96.94  |     |      | .48  | 2.34 |       |       | 55                           |
| 8   | 96.71  |     |      | .66  | .50  | 1.88  |       | 1109                         |
| 9   | 66.00  |     |      |      | 5.00 | 1.5   | 27.50 | 4                            |
| 10  | 66.00  |     | 1.00 |      | 5.00 | 1.5   | 26.50 | 48                           |
| 11  | 98.25  |     |      | 1.50 | .25  |       |       | 4234                         |
| 12  | 97.00  |     | 1.00 | 1.75 | .25  |       |       | 1058                         |
| 13  | 95.00  |     |      |      |      | 5.00  |       | 34½                          |
| 14  | 94.00  |     | 1.00 |      |      | 5.00  |       | 90                           |
| 15  | 97.50  |     |      | 2.50 |      |       |       | ½                            |
| 16  | 99.00  |     |      | 1.00 |      |       |       | ½                            |
| 17  | 98.00  |     |      |      | 2.00 |       |       | ½                            |
| 18  | Copper |     |      |      |      |       |       |                              |
| 19  | 89.90  |     |      | .10  |      | 10.00 |       | 16                           |
| 20  | 89.75  |     |      | .25  |      | 10.00 |       | 201                          |
| 21  | 89.50  |     |      | .50  |      | 10.00 |       | 652                          |
| 22  | 88.75  |     |      | .25  |      | 10.00 | 1.00  | 187                          |
| 23  | 88.50  |     |      | .50  |      | 10.00 | 1.00  | 407                          |

45 of the cadmium-bearing copper base alloys under stress in steam. My tests show other elements such as manganese, nickel, tin and arsenic, and combinations of these elements materially aid in preventing or inhibiting the action of 50 steam and/or gases in steam on copper and copper base alloys, and although we recognize the beneficial effects of the presence in certain copper base alloys for service in steam of such elements as manganese, nickel, tin and arsenic, I 55 have discovered and demonstrated that cadmium is the most beneficial in a great many instances, and even improves the corrosion resistance to steam and/or gases when used with these elements. The following are examples.

60 Cadmium added to commercial copper  
Cadmium added to copper-tin alloys  
Cadmium added to copper-nickel-aluminum alloys  
65 Cadmium added to copper-nickel-aluminum-zinc alloys  
Cadmium added to copper-silicon-manganese alloys  
Cadmium added to copper-nickel-silicon alloys  
70 Cadmium added to copper-nickel alloys  
Cadmium added to copper-silicon alloys  
Cadmium added to copper-aluminum alloys

The cadmium is ordinarily in amount from 0.01% to approximately 1.50% of the alloy, although it may be as high as 3%, if desired.

In many instances apparatus fabricated of these cadmium-bearing copper base alloys may need to be joined by welding. It has been found that such welds can be and are preferably made from similar cadmium-bearing welding or filler rods, for it is important that welding joints be 5 as resistant to the disintegrating action of steam as the metals welded.

A characteristic of a number of these alloys is a reddish surface film noticeable after annealing or heating, especially on the surface of the lighter nickel-bearing alloys. This film appears to afford some protection against intercrystalline parting or corrosion.

In casting the aforesaid copper base cadmium-bearing alloys the cadmium may be added as the metal or in any other suitable form of alloy. In other words it may be added as in usual casting shop practice. A satisfactory way is to

add it as master alloy, say for example of 90% 45 copper and 10% cadmium. The resultant alloy may be cast in any suitable molds. Said castings may then be rolled, forged, hammered, drawn, extruded, etc. either hot or cold, and in most instances both hot and cold, into various 50 forms, such as sheets, bars, rods, wire tube, and the like, by methods now well known and practiced in the copper alloy industry.

Some of the uses to which the cadmium-bearing copper base alloys may be put include conductors of electricity and of heat, particularly where steam is present, condenser tubes, expansion joints and the devices of the sort in steam lines, steam regulating devices or controls, corrugated seamless tubes, and flexible metal hose, 60 bellows, diaphragms and other parts of steam or water controls and power devices, valves or traps, heater tubes, steam conductors, and reservoirs, tanks, vats and other containers of liquids at steaming temperatures, steam turbine blades 65 and other parts, and all apparatus particularly designed for steam service or to resist the corrosive and disintegrating action of steam.

In the accompanying drawing are shown examples of various articles for use in steam and hot 70 water service which are greatly improved for this service by my invention, as their life both stressed and unstressed when used in contact with steam or hot water is greatly increased by the use of these alloys containing cadmium as this greatly 75

inhibits corrosion and disintegration due to the action of the steam and hot water and/or gases in steam.

In this drawing Fig. 1 is a longitudinal section of a pipe, tube or conductor which may be used for conducting steam and hot water;

Fig. 2 is a cross section thereof;

Fig. 3 is a longitudinal section of a portion of a bellows which may be used for expansion joints, controlled or regulating devices, etc. for steam and hot water service;

Fig. 4 is a cross section thereof;

Fig. 5 is a cross section of cupped, drawn or formed metal sheets telescoping each other and adapted for use in steam service and steam regulating devices;

Fig. 6 is a top plan view thereof;

Fig. 7 is a longitudinal section of an annular, corrugated, seamless tube which may be used in steam or hot water systems;

Fig. 8 is a transverse section thereof;

Fig. 9 is a partial longitudinal section and a partial side elevation of another type of a corrugated seamless tube;

Fig. 10 is a transverse section thereof;

Fig. 11 is a side elevation of a boiler or container for steam or hot water;

Fig. 12 is a transverse section of a flexible diaphragm;

Fig. 13 is a top plan view thereof;

Fig. 14 is a top section of a plane diaphragm;

Fig. 15 is a plan view thereof;

Fig. 16 is a partial longitudinal section and partial side elevation of another form of flexible metal tube or hose;

Fig. 17 is a transverse section thereof;

Fig. 18 is a flat sheet metal piece;

Fig. 19 is a similar strip curved to any desired shape; and

Fig. 20 is a perspective view of a tank or container.

The tube or conductor 21 of Figs. 1 and 2 may be of any ordinary cross sectional shape, and for steam and hot water service made of my improved alloy containing cadmium.

The flexible bellows 22 of Figs. 3 and 4 is of flexible sheet metal corrugated as shown and is adapted for use in expansion joints or as bellows forming the expanding and contracting element of regulating devices responsive to pressure.

The device of Fig. 5 comprises two cupped sections 23 and 24 cupped, drawn or formed from sheet metal sheets of this alloy and are assembled in telescoping relation so as to adjust the position under various pressures, etc. in regulating devices for steam and hot water systems. They may be connected to the system by suitable pipe connections to the nipples 25.

The corrugated seamless tube 26 of Fig. 7 is made of thin flexible metal and may be used for conducting steam and water and other similar uses. The corrugations in this particular form are annular.

The seamless tube 27 of Figs. 9 and 10 is similarly constructed except that the spirals run helically and may be used for conducting steam and

other uses the same as the tubes of Figs. 7 and 8.

The element 28 in Fig. 11 shows diagrammatically a boiler, tank or other container for steam or hot water, and may be constructed in any desired manner, such as riveted or welded sheets, 5 heads, etc.

The diaphragm 29 of Figs. 12 and 13 is made from a thin flexible sheet of metal alloy and may be corrugated as indicated at 30 and may be used for regulating devices, etc. 10

The diaphragm 31 of Figs. 14 and 15 is substantially the same except that it is plain instead of corrugated.

In Figs. 16 and 17 is shown a common type of helically wound interlocked flexible metal hose it 15 being formed of a strip 32 shaped at one side by bending inwardly and laterally as shown at 33 and placed between outwardly bent portion 34 of the opposite edge of the next adjacent convolution, so that these convolutions are inter- 20 locked and are capable of certain relative movement to permit flexing of the tube. They may be used for conducting steam or hot water between relatively movable elements of a system and in other locations as found desirable. 25

The flat plate 35 of Fig. 18 may be used for any desirable purpose or for making various elements of the steam or hot water system.

The same is true of the irregular shape 36 of Fig. 19. 30

The tank 37 shown in Fig. 20 may be of any suitable construction that shown having side walls 38 and end walls 39 and a bottom wall not shown.

These elements illustrated are shown merely 35 as examples of the large number of elements which may be improved by my invention whereby they have increased resistance to corrosion and disintegration when used in contact with steam and hot water.

In addition to imparting the resistance to corrosion and disintegration the cadmium also imparts resistance to "creep" (gradual elongation) under stress even at the elevated temperatures met with in use with hot water and steam. 40 45

My preferred invention is therefore an alloy intended principally for service in steam and characterized by the presence of cadmium from 0.01 to approximately 3.0%. This alloy is usually wrought, either hot or cold, or both, but may be used in the cast condition or in a weld or braze. 50

Having thus set forth the nature of my invention, what I claim is:

1. An element for use in conveying or distributing steam or hot water fabricated from copper 55 or a copper base alloy in which the tendency to intercrystalline parting in the metal is reduced by the incorporation of a small percentage of cadmium.

2. An element for use in conveying or distributing steam or hot water fabricated from a copper or a copper base alloy in which the tendency to intercrystalline parting in the metal is reduced by the incorporation of 0.01% to 3% cadmium. 60 65

CHARLES H. DAVIS.

CERTIFICATE OF CORRECTION.

Patent No. 2,034,561.

March 17, 1936.

CHARLES H. DAVIS.

It is hereby certified that error appears in the printed specification of the above numbered patent requiring correction as follows: Page 1, second column, line 23, for the word "indicates" read indicate; line 42, for "proportionally" read proportionally. The table, page 2, should be inserted between lines 17 and 18 of column 1; in the heading to the table, for "bar" read base, and in the table, test No. 18, strike out the dotted line in the last column and insert instead a zero; and that the said Letters Patent should be read with these corrections therein that the same may conform to the record of the case in the Patent Office.

Signed and sealed this 8th day of December, A. D. 1936.

Henry Van Arsdale  
Acting Commissioner of Patents,  
(Seal)